

# UNITED STATES PATENT OFFICE.

ROBERT C. HARTONG, OF AKRON, OHIO, ASSIGNOR TO THE GOODYEAR TIRE & RUBBER COMPANY, OF AKRON, OHIO, A CORPORATION OF OHIO.

## RUBBER MIX AND PROCESS OF COMPOUNDING RUBBER.

1,370,965.

Specification of Letters Patent.

Patented Mar. 8, 1921.

No Drawing. Original application filed March 30, 1917, Serial No. 158,525. Divided and this application filed January 30, 1919. Serial No. 274,017.

*To all whom it may concern:*

Be it known that I, ROBERT C. HARTONG, a citizen of the United States, residing at Akron, in the county of Summit and State 5 of Ohio, have invented a new and useful Improvement in Rubber Mix and Processes of Compounding Rubber, of which the following is a specification.

My invention relates to the art of compounding rubber and will be fully understood from the following specification.

In the manufacture of rubber products a large variety of compounding ingredients are employed and in every instance it is desirable to secure a uniform and homogeneous mixture of these ingredients, both with one another and with the rubber, in order that the vulcanized product may be of highest quality. My invention is particularly concerned with a method of procedure by which compounding ingredients may be incorporated into and disseminated through the rubber mix in the finest practical state of subdivision and in such a manner as to secure 20 true homogeneity. This end I find to be best attained by the use of a liquid carrier for the compounding ingredients.

It is a well understood fact that the action of a solvent liquid upon a solid is to 30 disintegrate that solid and break it up into excessively small particles, these particles when dispersed through the liquid being said to dissolve therein. For example it is believed that some substances of which the 35 soluble carbohydrate sugar may be taken as an illustration, disintegrate into their ultimate molecules in the presence of a sufficiently large volume of water, so that in a sugar solution the sugar exists in the most 40 extreme state of physical subdivision or dispersion of which it is capable. Other substances, such as glue for instance, when dissolved in water do not appear to be subdivided to the same extent as the sugar particles mentioned, but on the other hand they 45 enter into some species of combination with the water by which they become enormously swollen or distended and if subjected to a grinding action in this distended condition 50 may be more finely divided than is possible in handling the dry product. In still other instances there may be a disintegrating action by the solvent not approaching the disintegrating action effected in the case of the

sugar solution but nevertheless very decided, 55 unaccompanied by any noticeable combination of the solid with the solvent. Illustrations of this species of action are found in colloidal solutions of metals such as gold and platinum in water and in such materials as 60 arsenic sulfid, clay, and the like. Finally the solvent may have comparatively little disintegrating power upon the solid but nevertheless still shows a distinct power of maintaining the solid in a fine state of subdivision or dispersion when this subdivision has been effected, or at least of enormously 65 decreasing the rate of association of the particles of a finely divided substance. Thus for example when coarse materials of the 70 nature of barytes are suspended in water, each individual particle is retained in its separate state, agglomeration of the particles being prevented so long as the water is present in reasonable amounts. 75

It is therefore true that a carrier liquid is in general useful to some extent, either in effecting disintegration of a solid substance or preventing or retarding the reassociation of disintegrated particles which have been 80 reduced to a fine state of subdivision by any means. From this standpoint alone therefore the use of a carrier liquid is advantageous in the compounding of rubber. A further important advantage arises from the 85 fact that the liquid carrying the solid with it may be disseminated through the rubber with a relatively small amount of mechanical working, thereby avoiding the breaking down and loss of tensile strength of the rubber which results from the excessive working sometimes necessarily resorted to in order to effect thorough dissemination of a 90 solid compounding ingredient. The carrier liquid is also of particular advantage in the 95 case of solid compounding ingredients which form true solutions such as the sugar solution mentioned, or which form colloidal solutions either as emulsion colloids or as suspension colloids and where relatively small 100 percentages of the particular compounding ingredients are employed. By the increase in bulk or volume resulting from the action of the carrier liquid the difficulty of effecting thorough dissemination of these relatively small percentages through the mass of 105 the rubber mix is substantially lessened.

I have found that for the majority of

- compounding materials employed in the manufacture of rubber, water forms the most desirable carrier liquid, both because of its cheapness and because of the fact that it does not act upon the rubber in the mix. It must be understood, however, that other carrier liquids may be employed without departure from the basic principles of my invention.
- 10 After the mix has been satisfactorily compounded the water or other carrier liquid must be removed, it being well known that any large percentage of vaporizable matter such as water in the ordinary rubber mix is highly disadvantageous in that vapors are evolved during vulcanization and the vulcanized product is thereby rendered porous. I find that the water may readily be removed, however, either by vacuum drying or by the use of a current of air or other inert gas, the expense of the treatment being far outweighed by the advantages resulting from the use of the carrier liquid in compounding.
- 25 In the use of alumina as a compounding ingredient by ordinary methods employed for its dissemination through the mass it is difficult to secure satisfactory results. If, however, the alumina be suspended in water in the form of the hydrate  $(Al(OH)_3$ ), which may readily be produced in the vehicle by precipitation or other means well known in the chemical arts, this hydrate assumes a more or less colloidal state and is in a much finer state of subdivision or dispersion than any to which the oxid itself may be reduced. By incorporation of such an aqueous suspension of aluminum hydroxid in a rubber mix, I secure a perfectly homogeneous mass in which, after removal of the water, for example, by vacuum drying, the alumina is perfectly distributed in an exceedingly fine state of subdivision. On subsequent vulcanization the product shows in all its physical properties improvements indicating the more perfect nature of the mixing process.
- It is readily apparent that my invention is not limited to the specific material described, but may be utilized for the incorporation in the rubber mix of other metallic compounds and metals which may exist in the presence of a carrier vehicle as dispersed, suspended colloids. Thus other metallic hydroxids may be obtained as suspended colloids in water as may certain metals such as iron and lead. These materials cannot be secured in a form having commercial value as compounding ingredients by mechanical grinding to the finest possible powder. However, when such substances as these metallic hydroxids and metals are obtained in colloidal form in suspension, for example, in water or in dilute colloidal solutions of gelatin or other precipitative colloids and are added to the rubber, moisture being subsequently removed, they are homogeneously incorporated in an exceedingly fine state of dispersion and a very decided improvement in the quality of the finished product is secured.
- It will be understood that my invention is not dependent upon the soundness of the theories which have been stated in the present application nor is it limited to the specific materials or methods of manipulation named, excepting so far as such limitations are included within the terms of the accompanying claims.
- This application is a division of my prior application Serial No. 158,525, filed March 30, 1917.
- I claim:
1. The process of compounding rubber which consists in adding to rubber, water carrying in suspension hydroxid of aluminum, mixing the water and aluminum hydroxid with the rubber, driving off the water, and heating the mix with a vulcanizing agent to effect vulcanization.
  2. A rubber mix containing rubber and aluminum hydroxid in finely dispersed form homogeneously distributed therethrough.

In witnesses whereof, I have hereunto signed my name in the presence of two subscribing witnesses.

ROBERT C. HARTONG.

Witnesses:

L. M. HARTMAN,  
B. J. McDANEL.